

# UNITED STATES PATENT OFFICE.

HENRY E. LEPPER, OF CARSON, NEVADA.

## LUBRICATING COMPOUND.

SPECIFICATION forming part of Letters Patent No. 278,243, dated May 22, 1883.

Application filed March 26, 1883. (No specimens.)

*To all whom it may concern:*

Be it known that I, HENRY E. LEPPER, a citizen of the United States, residing at Carson, in the county of Ormsby and State of Nevada, have invented certain new and useful Improvements in Lubricating Compounds; and I do hereby declare the following to be a full, clear, and exact description of the invention, such as will enable others skilled in the art to which it appertains to make and use the same.

My improved lubricating compound consists of beeswax, resin, paraffine-oil, lard-oil, and tallow, combined in about the proportions hereinafter stated—that is to say: beeswax, one part; resin, one part; paraffine-oil, one part; lard-oil, three parts; tallow, six parts. These ingredients are melted and thoroughly mixed in any suitable manner.

A lubricant composed of these ingredients will not be readily decomposed by heat or friction, and may be used successfully for all lubricating purposes.

What I claim as my invention, and desire to secure by Letters Patent, is—

The herein-described composition of matter, to be used as a lubricant, consisting of beeswax, resin, paraffine-oil, lard-oil, and tallow, in about the proportions specified.

In testimony whereof I affix my signature in presence of two witnesses.

HENRY E. LEPPER.

Witnesses:

M. H. YERINGTON,  
ALFRED LILIENFELD.